

## UNITED STATES PATENT OFFICE

KARL HEINRICH WOLMAN, OF BERLIN-GRUNEWALD, AND HANS PFLUG, OF BERLIN-STEGLITZ, GERMANY, ASSIGNEES TO GRUBENHOLZ-IMPRÄGNIERUNG, G. M. B. H., OF CHARLOTTENBURG, GERMANY

## WOOD PRESERVATIVE

No Drawing. Application filed August 25, 1927. Serial No. 215,529.

It is known to treat wood with aqueous solutions of salts having a preserving action for the purpose of protecting it from destruction by vegetable and animal pests. For this purpose use is made, for example, of aqueous solutions of copper sulphate, zinc chloride and, particularly in recent times nitrated phenols. All these preservatives have certain disadvantages. The copper sulphate solutions has an insufficiently strong fungicidal action and cannot be employed in iron impregnating vessels. Zinc chloride, also, is not sufficiently effective; furthermore it is too easily washed out of the wood by atmospheric deposits and it attacks the iron armourings of the wood, forming hydrochloric acid. Nitrated phenols or salts thereof have the drawback that they are more or less explosive and that their aqueous solutions decompose and corrode the iron of the vessels in which the wood is impregnated.

The present invention enables these drawbacks to be avoided. The invention consists in employing amino-phenol salts of those acids which themselves have a fungicidal action. For instance use may be made of the water-soluble hydrofluoric acid, fluosilicic acid, arsenious acid and arsenic acid salts of amino derivatives of phenols, cresols, xylols or naphthols. The invention is not limited to the use of particular acids or particular aminophenols, but all suitable acids and aminophenols, i. e., for instance mono-, di-, or polyaminophenols, may be used. The said salts of aminophenols are not explosive and are very highly effective, so that even when used in a small quantity, they afford a thorough and permanent protection to the wood. Instead of phenol derivatives containing only amino groups, use may also be made of those aminophenols which, in addition to the amino groups, contain one or more nitro groups. It has also proved advisable to add to the salts of aminophenols or nitro-aminophenols, water-soluble salts, for in-

stance alkali salts, of those acids which are used to form salts with the aminophenols. For instance, sodium fluoride may be added to the fluorides of aminophenols, or potassium arsenite to the arsenites of aminophenols, and so on. These additions increase the stability of the solutions and also help to protect the wood by their own fungicidal action. Mixtures of several aminophenols, and also mixtures of several of the additions referred to, may also be employed. It is also possible to add to the described preservatives other compounds which have a preserving action or which reduce the inflammability of the wood and finally also compounds which protect the iron from corrosion.

The solutions of the new wood preservative may be used in any suitable manner for impregnating the wood. The latter may be coated with the solutions or steeped in the solution in open receptacles or, as is most advisable, the solution may be introduced into the wood in closed iron vessels with the employment of vacuum and pressure.

For example, 1 kg. of arsenite of para-aminophenol, which is obtained by boiling aminophenol with an excess of aqueous arsenic acid and allowing the resulting compound to crystallize out, is dissolved in 100 kg. of water and this solution is used for coating or impregnating wood.

Alternatively 0.4 kg. of the fluoride of 2,4-nitroaminophenol is dissolved in 100 kg. water and the wood is treated with this solution, for instance by coating. The fluoride of 2,4-nitroaminophenol is obtained by dissolving 2,4-nitroaminophenol in an excess of aqueous hydrofluoric acid, evaporating the solution, dissolving the residue in hot water and allowing the solution to crystallize.

As a further example, 0.2 kg. of the fluoride of 2,4-nitroaminophenol and 1 kg. of sodium fluoride may be dissolved in 100 kg. water and the wood treated with this solution in

closed vessels, a vacuum and pressure being employed.

What we claim is:—

1. A wood preservative, consisting of alkaline fluorides and compounds of nitroamino-phenols with hydrofluoric acid.
- 5 2. A wood preservative, consisting of sodium fluoride and compounds of nitro-aminophenols with hydrofluoric acid.
- 10 In testimony whereof we have signed our names to this specification.

**KARL HEINRICH WOLMAN.**  
**DR. HANS PFLUG.**

15

20

25

30

35

40

45

50

55

60

65